

H. VON FORSTER.

MANUFACTURE OF COLD DRAWN SEAMLESS TUBES.

APPLICATION FILED JULY 16, 1914.

1,205,292.

Patented Nov. 21, 1916.

3 SHEETS—SHEET 1.



Witnesses:

R. W. Cadairi.

*S. Denning*

Inventor

Hermann von Forster

*by*  
Foster, Sherman, Watson & Gitt  
Attorneys

1,205,292.

H. VON FORSTER,  
MANUFACTURE OF COLD DRAWN SEAMLESS TUBES,  
APPLICATION FILED JULY 16, 1914.

Patented Nov. 21, 1916.  
3 SHEETS—SHEET 2.



*Fig. 4.*  
NEW

Witnesses:

L. W. Cedar  
A. C. Denney,

Inventor:  
Hermann von Forster  
by  
Foster Freeman Hartman & Hart  
Attorneys

1,205,292.

H. VON FORSTER.  
MANUFACTURE OF COLD DRAWN SEAMLESS TUBES.  
APPLICATION FILED JULY 16, 1914.

Patented Nov. 21, 1916.

3 SHEETS—SHEET 3.

Fig. 5.



Fig. 6.



Witnesses:

L. W. Cadairi,

Richenay.

Inventor  
Hermann von Forster  
By  
Foster-Fischer-Hallinan, Attorneys.

# UNITED STATES PATENT OFFICE.

HERMANN VON FORSTER, OF FRANKFORT-ON-THE-MAIN, GERMANY.

## MANUFACTURE OF COLD-DRAWN SEAMLESS TUBES.

1,205,292.

Specification of Letters Patent. Patented Nov. 21, 1916.

Application filed July 16, 1914. Serial No. 851,364.

To all whom it may concern:

Be it known that I, HERMANN VON FORSTER, a subject of the German Emperor, residing at 32 Roseggerstrasse, Frankfort-on-the-Main, Germany, have invented certain new and useful Improvements in the Manufacture of Cold-Drawn Seamless Tubes, of which the following is a specification.

This invention relates to certain improvements in the manufacture of cold-drawn seamless metal tubes of any desired cross-section.

Hitherto it has been usual to subject a comparatively thick and irregular hollow blank, prepared by rolling, hammering, casting or the like, on a draw-bench in a cold state to the action of dies which reduce the thickness of the blank to form a comparatively thin and uniform tube. The drawing is effected either by fitting the blank upon a short mandrel and pushing it over the mandrel or by fitting it upon a mandrel of a length equal to the length of the finished tube and passing the blank and mandrel together through the dies. The first-mentioned process has the advantage that the tube frees itself from the mandrel during the drawing operation whereas the second-mentioned process allows a greater reduction of the thickness of the tube or blank in each pass, thus necessitating a less number of passes. In the latter case however the tube has to be specially removed from the mandrel. In the aforesaid processes however the material after the first few passes attains such a degree of hardness that it is impossible to continue the drawing operation and it has therefore been usual to resort to annealing after the first few passes in order to remove the hardness of the material and to restore its ductility which had been previously so far reduced by the previous drawing operation that the ultimate state of fluidity almost approached breaking strength. After annealing, the partly finished tube was then brought on to the draw-bench and the drawing operation continued. The annealing process occupied a considerable time and consequently the manufacture of the tubes was a slow process. The cost was also increased by the transport between the annealing furnace and the draw-bench.

The object of the present invention is to considerably facilitate the manufacture

of cold-drawn seamless metal tubes and to dispense with the annealing process.

According to the present invention the hollow blank is elongated and its thickness reduced in a plurality of immediately succeeding passes which reduce the blank substantially uniformly, each pass reducing the thickness of the blank substantially the same amount.

In order that the invention may be more clearly understood reference will be herein-after made to the accompanying drawings, whereon—

Figure 1 is a diagram representing the old method of cold-drawing seamless metal tubes and Fig. 2 a diagram representing the method according to the present invention. Figs. 3 and 4 are diagrams showing the tensile stress and the ultimate breaking and ductile strength of the tube during the processes of manufacture represented in Figs. 1 and 2 respectively. Fig. 5 is a side view of a draw-bench for carrying out the improved method and Fig. 6 is a plan view thereof.

On reference to Fig. 1 it will be seen that in the old method the complete drawing operation took place in a series of stages between which an annealing process intervened, the material being subjected to a considerable pull in the first pass of each stage and to one or two considerably weaker pulls after the first pass and before annealing. The opinion hitherto prevailed that the ductility of the material was so far exhausted when the ultimate state of fluidity had approached the ultimate breaking strength that further change of form could not be effected with practical economy. This appeared to be proved by the fact that the tubes fractured on further elongation. According to the present invention the drawing operation is carried out continuously, without intermediate annealing, the blank being subjected to a larger number of uniformly decreasing or almost uniformly decreasing weaker pulls in immediate succession. The gradual reduction in the tensile strain is indicated in Fig. 2.

In order to show the possibility of carrying out the present invention it may be explained that the considerable reduction in the thickness of the blank in the old process causes immediate hardness of the material so that the ultimate state of fluidity very

rapidly approaches the ultimate breaking strength and renders the further operation difficult. This will be apparent from Fig. 3, wherein  $t$  represents the tensile stress,  $d$  the ultimate ductile strength, and  $f$  the ultimate breaking strength. In the new process, on the contrary, hardness occurs more on the surface whereas the interior retains its ductility for a considerably longer period of time as will be apparent from Fig. 4. Whereas it was found uneconomical in the old process to make further small changes in the form of the blank it has been found in the present process which is based on the employment of a considerable number of passes, that in this continuous process slight changes of form such as were hitherto unpractical have been found economical. The possibility of employing such a large number of individual passes, say 20 to 30 or more, is further supported by the fact that in the continuous process each pass may immediately succeed the foregoing pass. In this case the heat generated by the change in form is not lost as in the old process where the work takes place periodically but is utilized and increased by the immediate succession of the passes. This heat serves in the first place to reduce the hardness and brittleness naturally occurring on the surface and also to reduce the increase of the ultimate state of fluidity toward the ultimate breaking strength. The manufacture is also considerably simplified by the present invention for whereas the tubes were manufactured hitherto in stages, each stage being interrupted by the annealing process which occupied such a considerable length of time, the tube can now be manufactured in one stage without being transported. This of course considerably reduces the cost and time as well as the works fittings and enables the tubes to be turned out with great rapidity.

Referring now to Figs. 5 and 6 of the drawings,  $a$  designates the legs of the draw-bench, and  $b$  the blank which is fitted upon a mandrel  $c$  reduced in thickness at the right hand end so as to receive the smallest die. The blank is fitted over the thicker part of the mandrel up to the shoulder thereon at the junction therewith of the reduced part. Mounted on the bed  $e$  of the draw-bench is a plurality of die holders  $g$  in which the dies  $f$  are mounted, the die holders  $g$  being slidable over the reduced part of the mandrel  $c$ . The die holders  $g$  are adapted to be moved in turn up to the shoulder on the mandrel  $c$ . One of the die holders  $g^1$  is shown in this position ready for the drawing operation.

Mounted on the power shaft  $i$  is a crank  $k$  which transmits motion to a forked or parallel lever  $m$  through the connecting rod  $l$ . Beneath the bed of the machine is a runway

$n$  which may be dovetailed to receive a slide  $o$  which carries two projecting pins  $p$  and  $q$  at each side. The pin  $p$  engages a slot  $m^1$  in the lever  $m$  so that the slide  $o$  is reciprocated in the runway  $n$  by the lever  $m$ . 70

Pivoted on the pins  $q$  are fingers  $r$  under the action of springs  $t$  between the fingers  $r$  and a projection  $s$  on the slide  $o$ . In the position shown the fingers  $r$  move the first die-holder  $g'$  over the blank  $b$  and as soon as 75 the crank  $k$  has reached its other dead position the lever  $m$  and slide  $o$  return, the fingers  $r$  leaving the die-holder  $g'$  at the rear end of the machine. In the meantime the next die-holder  $g$  has been moved up to the shoulder on the mandrel  $c$  so that the fingers  $r$  pass beneath the pins  $h$  of this die-holder and engage behind the same under the action of the springs  $t$  so that the parts are then in position for the next drawing operation. 80 85 This process is repeated until the whole of the dies have been moved over the blank.

In the machine described the comparatively light dies alone require to be moved whereas the blank remains stationary. This 90 arrangement is found preferable in carrying out the present invention.

It will of course be understood that the die-holders may be dispensed with and any other suitable mechanism provided for actuating the dies.

Where the total reduction which the blank is required to undergo is very considerable it may be found desirable to subdivide the process into stages, the blank being reduced 100 on one machine according to the present process to a certain thickness and then reduced still further on a second draw-bench with or without intermediate annealing. 105

I claim:

1. The improvement in the manufacture of cold-drawn seamless thin-walled metal tubes, which consists in continuously drawing out a cold hollow blank to a finished thin tube in substantially uniform stages immediately succeeding each other. 110

2. The improvement in the manufacture of cold-drawn seamless thin-walled metal tubes, which consists in drawing out a cold hollow blank to a thin tube in an uninterrupted series of substantially uniform drawing operations. 115

3. The improvement in the manufacture of cold-drawn seamless thin-walled metal tubes, which consists in subjecting a cold hollow blank on the draw-bench to as many passes in close succession as will suffice to reduce it to a finished thin tube. 120

4. The improvement in the manufacture of cold-drawn seamless thin-walled metal tubes, which consists in drawing a cold hollow blank in close succession through as many dies of slightly and substantially uniformly decreasing diameters as will suffice to reduce it to a finished thin tube. 125 130 135

5. The improvement in the manufacture of cold-drawn seamless thin-walled metal tubes, which consists in drawing out a cold hollow blank in close succession between a mandrel and as many dies of slightly and substantially uniformly decreasing diameters as will suffice to reduce the blank to a finished thin tube.
6. The improvement in the manufacture 10 of cold-drawn seamless thin-walled metal tubes, which consists in passing in close succession over a cold hollow blank mounted on a mandrel, as many dies of slightly and substantially uniformly decreasing diameters as 15 will suffice to reduce the blank to a finished thin tube.
7. The improvement in the manufacture of cold-drawn seamless thin-walled metal tubes, which consists in mounting a hollow blank on a mandrel and passing over it in close succession as many dies of slightly and substantially uniformly decreasing diameters as will suffice to reduce the blank to a finished thin tube.

In testimony whereof I affix my signature 25 in presence of two witnesses.

HERMANN VON FORSTER.

Witnesses:

JEAN GRUND,  
CARL GRUND.